

## UNITED STATES PATENT OFFICE

1,979,254

## LEAD-SODIUM ALLOY

Frederick Baxter Downing, Carneys Point, and  
 Louis S. Bask, Penns Grove, N. J., assignors to  
 E. I. du Pont de Nemours & Company, Wil-  
 mington, Del., a corporation of Delaware

No Drawing. Application January 25, 1934,  
 Serial No. 708,248

2 Claims. (Cl. 75—1)

This invention relates to an improvement in the production of lead alkyls by the reaction of alkyl halides upon a lead sodium alloy, and more particularly to the alloys employed in such process.

In the process as ordinarily practiced at the present time a lead sodium alloy consisting of 90% lead and 10% sodium is reacted with ethyl chloride to form a dry reaction mass containing lead alkyl absorbed by finely divided lead, sodium halide and an appreciable amount of undecomposed alloy. The lead alkyl is recovered from the mass by drowning in water and distilling out the lead alkyl by means of steam. By the use of such process, employing ethyl chloride, yields of from 83% to 85% of tetra ethyl lead have been obtained in the laboratory, with amounts of about 5% to 10% of the alloy left undecomposed. Such undecomposed sodium tends to cause trouble in the recovery of the alkyl lead compounds by steam distillation, due to the fact that the undecomposed sodium reacts with the water in which the reaction mass is drowned with the result that the metallic lead tends to form large balls, cakes or rings which lower the recovery of the alkyl lead and are removed from the still only with great difficulty. In order to eliminate this balling of the lead, as much as possible, it has been necessary to add a protective agent such as, for example, thiocarbanilide or a dispersing agent such as engine oil, or both, to the reaction mass during distillation. However, these expedients have not proved to be entirely satisfactory as a large percentage of the distillations give trouble even in the presence of these substances.

An object of the present invention is to provide a process wherein these difficulties are eliminated. A further object is to provide a new composition of matter in the nature of an alloy to be used in such process which composition of matter is substantially completely decomposed during the reaction and has no tendency to cause balling or caking of the metallic lead. Still further objects are to provide a new composition of matter and to advance the art. Other and further objects will appear hereinafter.

These objects may be accomplished according to our invention which comprises substituting for a small proportion of the lead, in the lead sodium alloy of the process as heretofore practiced, a small amount of magnesium. We have found that when amounts of magnesium varying from 0.05% to 1.0% of the weight of the alloy is substituted for an equivalent weight of the lead in the preparation of the alloy and such new composition of matter is used in the manufacture

of lead alkyl compounds, higher yields of the lead alkyl compounds result, the composition is more completely decomposed during the reaction, and agglomeration of the lead particles during distillation is practically eliminated without requiring the use of a protective or dispersing agent. For example, when such composition of matter is employed in the production of tetra ethyl lead, yields of from about 85% to 88% are obtained and the amount of undecomposed composition in the reaction mass at the completion of the reaction amounts to from 4% to 9%, both the yield of tetra ethyl lead and the amount of undecomposed composition depending upon the amount of magnesium present in the composition employed. It has been found that as little as 0.1% of magnesium in the composition is sufficient to practically eliminate all agglomeration of lead particles during the distillation, which appears to be due to the fact that a much more complete reaction is obtained with less undecomposed composition present in the reaction mass. However, we preferably employ from about 0.15% to 0.4% of magnesium as such amount gives most satisfactory results.

In order to more clearly point out our invention and illustrate the preferred mode in which we contemplate carrying the same into effect, the following examples are given:

*Example 1.*—One hundred (100) grams of a lead-sodium alloy containing 90% lead and 10% sodium by weight, equivalent to equal molecular proportions of the two metals, were reacted with 50 cc. of ethyl chloride in a small pressure autoclave in a water bath of 75° C. for 5 hours. The resultant reaction mass was drowned in 500 cc. of water and the lead ethyl distilled off, with steam. The weight of lead ethyl recovered was 29.2 grams, equivalent to 84.3% yield, based on the sodium.

The unreacted sodium which was present as sodium hydroxide in the residue from the steam distillation was determined by titration with standard acid solution and the results calculated as sodium. This unreacted sodium was found to be 0.51 grams or 5.1%.

*Example 2.*—One hundred (100) grams of magnesium bearing lead sodium alloy consisting of 89.6% lead, 10% sodium and 0.4% magnesium were reacted with 50 cc. of ethyl chloride and the lead ethyl recovered in the same manner as recited in Example 1. The yield of the lead ethyl was found to be 30.98 grams or 88.1% based on the sodium.

No unreacted sodium was present in the reac-

80

85

70

75

80

85

90

95

100

105

110

tion mass as shown by the fact that the residue from the steam distillation to remove the lead tetra ethyl, was neutral to phenol phthalein.

The results obtainable by varying the amounts 5 of lead and magnesium in the composition are shown in the following table:

| 10 | Alloy        |            |            | Yield based on sodium percent of theory | Undecomposed alloy percent |
|----|--------------|------------|------------|-----------------------------------------|----------------------------|
|    | Lead percent | Na percent | Mg percent |                                         |                            |
| 15 | 90           | 10         | 0          | 84.3                                    | 5.1                        |
|    | 89.9         | 10         | 0.1        | 86.2                                    | 4.2                        |
|    | 89.8         | 10         | 0.2        | 87.3                                    | 2.5                        |
|    | 89.7         | 10         | 0.3        | 88.0                                    | 1.0                        |
|    | 89.6         | 10         | 0.4        | 88.1                                    | 0.0                        |
|    | 89.5         | 10         | 0.5        | 87.0                                    | 0.0                        |
|    | 89.0         | 10         | 1.0        | 86.0                                    | 0.0                        |

Although the use of about 0.4% of magnesium 20 in the composition appears to be most desirable from a theoretical standpoint, we have found that, for practical purposes, the use of from about 0.15% to 0.2% of magnesium is preferable as larger amounts introduce certain problems into

25

30

35

40

45

50

55

60

65

70

75

the manufacture of the composition and the recovery of the alkyl lead compounds.

While, in the above examples, we have specifically referred to the reaction of the alloy with ethyl chloride, it is to be understood that our novel alloy may be employed in the production of lead alkyls generally, with similar results. Many variations and modifications in the process as described will readily appear to those skilled in the art without departing from the spirit of our invention. Accordingly, the scope of our invention is to be limited solely by the appended claims construed as broadly as is permissible in view of the prior art.

We claim:

1. A composition of matter comprising 10% sodium, 89.95% to 89.00% lead and 0.05% to 1.00% magnesium.

2. A composition of matter comprising 10% sodium, from about 89.85% to 89.80% lead and from about 0.15% to 0.20% magnesium.

FREDERICK BAXTER DOWNING.  
LOUIS S. BAKE.

80

85

90

95

100

105

110

115

120

125

130

135

140

145

150